

June 18, 1968

W. B. F. MACKAY ET AL

3,388,986

HIGH SPEED TOOL STEEL

Filed Aug. 9, 1965

3 Sheets-Sheet 1



July 18, 1968  
Inventors  
William B. F. Mackay  
Robert B. Carson  
By Cushman, Nichols Cushman  
Attorneys

June 18, 1968

W. B. F. MACKAY ETAL

3,388,986

HIGH SPEED TOOL STEEL

Filed Aug. 9, 1965

3 Sheets-Sheet 2



FIG. 2

William B. F. Mackay  
Robert G. Carson  
By Cushman, Darby & Cushman  
Attorneys

June 18, 1968

W. B. F. MACKAY ET AL

3,388,986

HIGH SPEED TOOL STEEL

Filed Aug. 9, 1965

3 Sheets-Sheet 3



FIG. 3

William B. F. Mackay  
Robert J. Carson  
By Cushman, Darby & Cushman  
Attorneys

## 1

3,388,986

### HIGH SPEED TOOL STEEL

William B. F. Mackay, 21 Haist Road N., and Robert O. Carson, 81 Carboro Road, both of Fonthill, Ontario, Canada

Filed Aug. 9, 1965, Ser. No. 478,116

Claims priority, application Canada, June 4, 1965,  
932,496

4 Claims. (Cl. 75—126)

#### ABSTRACT OF THE DISCLOSURE

A high speed tool steel which in its hardening state has improved hardness suitably of the order of  $R_c$  70 hardness and thus improved wear resistance as well as improved toughness which steel consists of, on a percentage basis, 1.15 to 1.25 carbon, 4.00 to 4.5 chromium, 4.25 to 5.00 tungsten, 1.85 to 2.15 vanadium, 6.75 to 7.75 cobalt, 7.00 to 8.00 molybdenum, .20 to .40 manganese and .15 to .45 silicon, the balance being iron and residual impurities.

This invention relates to a new and improved steel composition and more particularly to a steel composition especially adapted for tool steels employed in high speed operations.

Among the properties which are desired for high speed tool steels are versatility, low ingot cost, suitable grindability, workability and response to heat treatment, and adequate tool life as related to heavy cutting and high speed machining and measured in terms of red hardness and abrasion resistance. Tungsten, molybdenum, vanadium, chromium and cobalt are the alloying elements found in these steels.

It is an object of this invention to provide a tool steel having high speed machining features superior to present steel compositions while still maintaining properties of versatility, suitable grindability, and workability and adequate response to heat treatment.

Other objects of the invention will become apparent from the description to follow:

The objects of this invention are attained in a tool steel having the following percentage composition:

|    |           |
|----|-----------|
| C  | 1.15—1.25 |
| Cr | 4.00—4.50 |
| W  | 4.25—5.00 |
| V  | 1.85—2.15 |
| Co | 6.75—7.75 |
| Mo | 7.00—8.00 |
| Mn | .20—.40   |
| Si | .15—.45   |

The balance iron plus residual impurities.

Some preferred percentage compositions were analysed as follows:

|     | C    | Mn  | Si  | P    | S    | Cr   | W    | V    | Mo   | Co   |
|-----|------|-----|-----|------|------|------|------|------|------|------|
| (1) | 1.20 | .30 | .40 | .014 | .010 | 4.33 | 4.49 | 2.02 | 7.62 | 7.34 |
| (2) | 1.20 | .25 | .40 | .013 | .011 | 4.34 | 4.57 | 2.07 | 7.60 | 7.20 |
| (3) | 1.22 | .29 | .42 | .014 | .010 | 4.32 | 4.52 | 2.02 | 7.64 | 7.34 |

The balance iron plus residual impurities.

## 2

Phosphorus and sulfur are considered as impurities at their low levels, the manganese being employed to reduce the harmful effects of sulfur on the hot workability of the steel.

5 A preferred heat treatment of the steel includes a pre-heat step of 1500—1550° F. followed by hardening at 2175—2225° F. with a recommended temperature being 2200° F. The material is then tempered at from 950—1200° F. with maximum hardness produced by a triple temper at 975—1025° F. with 2 hours of each temper.

An induction heat (H245) having the composition in preferred analysis No. 1 was melted, cast and processed to tool bit size for a comparative evaluation with the tool steel (H248) described in U.S. Patent 2,996,376.

15 This latter composition analysed as follows:

|    |      |
|----|------|
| C  | 1.12 |
| Mn | 0.31 |
| Cr | 4.32 |
| W  | 6.58 |
| V  | 1.99 |
| Mo | 3.83 |
| Co | 4.70 |

Some of the test data are graphically illustrated in FIG-25 URES 1-3.

#### TOUGHNESS COMPARISONS

Un-notched izods were prepared by fully heat treating oversize bars, then carefully finish grinding in the hardened condition using a soft wheel and low metal removal rate. All specimens were magnafluxed prior to testing.

The results are shown below and it will be noted that H245 is marginally superior to H248.

| Heat No. | Hardness | Un-notched Izod Impact Strength Values | Average Izod |
|----------|----------|----------------------------------------|--------------|
| H245     | 69.5     | 6-6-22.5-5-5-9-6-13-22-----            | 10.5         |
| H248     | 68.5     | 11-8-8-11-10-9-----                    | 9.5          |

#### TOOL LIFE TESTS

Four sets of tool steels were cut from  $\frac{3}{8}$ " square annealed stock. Two sets which were used corresponded to the analysis of H245 and H248. The other two tool steels analysed as follows:

|               | C    | Mn  | Si  | Cr   | W     | V    | Mo   | Co   |
|---------------|------|-----|-----|------|-------|------|------|------|
| A.1.S.1. T-15 | 1.25 | .30 | .39 | 4.25 | 10.00 | 4.30 | 2.50 | 5.50 |
| A.1.S.1. M-34 | .90  | .30 | .25 | 3.75 | 1.45  | 2.05 | 8.70 | 8.25 |

50 The tools ground from these grades had the following dimensions:

|                         |         |      |
|-------------------------|---------|------|
| Back rake               | degrees | 0    |
| Side rake               | do      | 10   |
| Side cutting edge angle | do      | 15   |
| End cutting edge angle  | do      | 5    |
| Relief                  | do      | 5    |
| Nose radius             | inches  | .030 |

A.1.S.1. H-11 was the material used to rate the tools. 60 A 3" diameter rod, 15" long of H-11 was quenched and tempered at 50  $R_c$ . Tool life was then measured against cutting speeds and the results are shown in FIG. 3. It will be observed that composition H245 has about twice the wear life of H248.

## HARDNESS COMPARISONS

(1) Room temperature hardness.—Samples about  $\frac{1}{2}'' \times \frac{1}{2}'' \times 1''$  were cut from the  $4\frac{1}{4}''$   $R_c$  sq. billets. Samples were salt hardened from 2100, 2150, 2200, 2250, 2300 and  $2350^{\circ}$  F., interrupt quenched at  $1050^{\circ}$  F. subsequently double tempered (2 hours each) at 1000, 1100 and  $1200^{\circ}$  F. The resultant hardness shown in FIGURES 1 and 2 indicate that the optimum hardening temperature is in the range  $2200$ – $2250^{\circ}$  F. Hardness of 68–69  $R_c$  was obtained on both compositions after hardening and then tempering at  $1000^{\circ}$  F. Applicants' analysis (H245) offers the most resistance to tempering, when hardened from  $2250^{\circ}$  F., which indicates superior hardness.

(2) Hot hardness.—A second hardness evaluation was determined by heat treating four samples: H245, H248, T-15 and M-34 and subjecting them to hot hardness tests. The heat treatment for H245, H248 and M-34 were as follows:

|                                                  | $^{\circ}$ F. |
|--------------------------------------------------|---------------|
| Preheat                                          | 1500–1550     |
| Salt harden                                      | 2190–2210     |
| Salt interrupt                                   | 1050          |
| Double draw 2 hrs. + 2 hrs. at $1025^{\circ}$ F. |               |

T-15 was given a heat treatment at somewhat higher temperatures as follows:

|                                                  | $^{\circ}$ F. |
|--------------------------------------------------|---------------|
| Preheat                                          | 1550–1600     |
| Salt harden                                      | 2225–2250     |
| Salt interrupt                                   | 1050          |
| Double draw 2 hrs. + 2 hrs. at $1025^{\circ}$ F. |               |

The results of the heat treatment tests were as follows:

| HOT HARDNESS                       |      |      |      |      |
|------------------------------------|------|------|------|------|
| Temperature at Test, $^{\circ}$ F. | H245 | H248 | M34  | T15  |
| RT                                 | 70.0 | 68.0 | 66.0 | 68.0 |
| 600                                | 62.7 | 62.5 | 60.5 | 61.8 |
| 800                                | 61.9 | 62.5 | 60.3 | 60.9 |
| 900                                | 61.0 | 59.5 | 59.3 | 58.3 |
| 950                                | 60.2 | 59.0 | 57.9 | 57.6 |
| 1,000                              | 59.5 | 58.0 | 57.4 | 56.7 |
| 1,050                              | 58.8 | 57.2 | 56.1 | 55.7 |

Grindability.—Samples of H245 and H248 were tested under the following conditions:

|                     |                                                                     |
|---------------------|---------------------------------------------------------------------|
| Machine             | Gallmeyer & Livingston<br>Surface Grinder.                          |
| Wheel specification | PA46–G8–V40.                                                        |
| Wheel size          | $7'' \times \frac{1}{2}'' \times 1\frac{1}{4}''$ .                  |
| Wheel speed         | 3500 r.p.m.                                                         |
| Material ground     | Various kinds as shown<br>below ( $2'' \times \frac{5}{8}''$ area). |
| Grinding fluid      | None—dry grinding.                                                  |
| Table speed         | 50 f.p.m.                                                           |
| Crossfeed           | .060" per table reverse.                                            |
| Infeed per pass     | .003".                                                              |
| Number of passes    | 150.                                                                |
| Dressing technique  | Open—.001" per pass until<br>wheel trued up.                        |

The following results were obtained:

| Material Number | Ground Rock-well | Metal Removed<br>Inches | Metal Removed<br>Grams | Wheel Loss,<br>Grams | Ratio of weight<br>of metal removed/weight<br>of wheel removed | Finish<br>M.I.,<br>RMS | Burn      | Load<br>on<br>Wheel | Check<br>on<br>Steel |
|-----------------|------------------|-------------------------|------------------------|----------------------|----------------------------------------------------------------|------------------------|-----------|---------------------|----------------------|
| H245            | C 67             | .437                    | 74.54                  | 5.90                 | 12.6                                                           | 85                     | Lt. Brown | Some                | No.                  |
| H248            | C 68             | .428                    | 71.14                  | 8.30                 | 8.6                                                            | 80                     | Tan       | Light               | No.                  |

It will be observed that on the basis of the above-noted tests, H245 is superior in hot hardness and grindability, and markedly better in tool life than H248, while still maintaining equivalent toughness to H248.

We claim:

1. A high speed tool steel having the following percentage composition:

|    |    |           |
|----|----|-----------|
| 10 | C  | 1.15–1.25 |
| 10 | Cr | 4.00–4.50 |
| 10 | W  | 4.25–5.00 |
| 10 | V  | 1.85–2.15 |
| 10 | Co | 6.75–7.75 |
| 15 | Mo | 7.00–8.00 |
| 15 | Mn | .20–.40   |
| 15 | Si | .15–.45   |

The balance iron plus residual impurities.

2. A high speed tool steel having the following percentage composition:

|    |    |      |
|----|----|------|
| 20 | C  | 1.20 |
| 20 | Mn | .30  |
| 20 | Si | .40  |
| 25 | P  | .014 |
| 25 | S  | .010 |
| 30 | Cr | 4.33 |
| 30 | W  | 4.49 |
| 30 | V  | 2.02 |
| 30 | Mo | 7.62 |
| 30 | Co | 7.34 |

The balance iron plus residual impurities, the latter including sulfur and phosphorus.

3. A high speed tool steel having the following percentage composition:

|    |    |      |
|----|----|------|
| 40 | C  | 1.20 |
| 40 | Mn | .25  |
| 40 | Si | .40  |
| 40 | P  | .013 |
| 40 | S  | .011 |
| 45 | Cr | 4.34 |
| 45 | W  | 4.57 |
| 45 | V  | 2.07 |
| 45 | Mo | 7.60 |
| 45 | Co | 7.20 |

50 The balance iron plus residual impurities, the latter including sulfur and phosphorus.

4. A high speed tool steel having the following percentage composition:

|    |    |      |
|----|----|------|
| 55 | C  | 1.22 |
| 55 | Mn | .29  |
| 55 | Si | .42  |
| 55 | P  | .014 |
| 55 | S  | .010 |
| 60 | Cr | 4.32 |
| 60 | W  | 4.52 |
| 60 | V  | 2.02 |
| 60 | Mo | 7.64 |
| 60 | Co | 7.34 |

The balance iron plus residual impurities, the latter including sulfur and phosphorus.

## FOREIGN PATENTS

164,412 8/1955 Australia.

## OTHER REFERENCES

## References Cited

## UNITED STATES PATENTS

2,147,122 2/1939 Emmons ----- 75—126  
2,996,376 8/1961 Nehrenberg et al. ---- 75—126  
3,113,862 12/1963 Harvey et al ----- 75—126  
3,259,489 7/1966 Hamaker et al. ----- 75—126

5 Metal Progress, Reprint from June 1963, "Rc 70 High Speed Steel," Handyside et al.  
Tool Steels, ASM, 1962, relied on pp. 674-678.  
ASM Transactions, vols. 32-33, 1944, pp. 431-445.

10 CHARLES N. LOVELL, *Primary Examiner.*